



US011680449B2

(12) **United States Patent**  
Atkins et al.

(10) **Patent No.:** US 11,680,449 B2  
(45) **Date of Patent:** Jun. 20, 2023

(54) **POLYCRYSTALLINE DIAMOND COMPACT WITH INCREASED LEACHING SURFACE AREA AND METHOD OF LEACHING A POLYCRYSTALLINE DIAMOND COMPACT**

(71) Applicant: **Halliburton Energy Services, Inc.**, Houston, TX (US)

(72) Inventors: **William Brian Atkins**, Houston, TX (US); **Gagan Saini**, The Woodlands, TX (US); **Grant O. Cook, III**, Spring, TX (US)

(73) Assignee: **Halliburton Energy Services, Inc.**, Houston, TX (US)

(\*) Notice: Subject to any disclaimer, the term of this patent is extended or adjusted under 35 U.S.C. 154(b) by 852 days.

(21) Appl. No.: **16/338,907**

(22) PCT Filed: **Nov. 2, 2016**

(86) PCT No.: **PCT/US2016/060063**

§ 371 (c)(1),  
(2) Date: **Apr. 2, 2019**

(87) PCT Pub. No.: **WO2018/084839**

PCT Pub. Date: **May 11, 2018**

(65) **Prior Publication Data**

US 2020/0040662 A1 Feb. 6, 2020

(51) **Int. Cl.**

**E21B 10/567** (2006.01)  
**E21B 10/573** (2006.01)

(Continued)

(52) **U.S. Cl.**

CPC ..... **E21B 10/5673** (2013.01); **B22F 3/24** (2013.01); **B22F 7/06** (2013.01); **C22C 26/00** (2013.01);

(Continued)

(58) **Field of Classification Search**

CPC ..... E21B 10/46; E21B 10/55; E21B 10/5735  
See application file for complete search history.

(56) **References Cited**

U.S. PATENT DOCUMENTS

5,054,246 A 10/1991 Phaal et al.  
8,316,969 B1 \* 11/2012 Bertagnolli ..... B01J 3/062  
175/428

(Continued)

FOREIGN PATENT DOCUMENTS

|    |                 |         |
|----|-----------------|---------|
| GB | 2465175         | 12/2010 |
| JP | 2010-516488     | 5/2010  |
| KR | 10-2008-0039491 | 5/2008  |

OTHER PUBLICATIONS

Examiner's Letter, Canadian Patent Application No. 3,037,846, dated Nov. 26, 2019, 5 pages.

(Continued)

*Primary Examiner* — Pegah Parvini

(74) *Attorney, Agent, or Firm* — Michael Jenney; C. Tumey Law Group PLLC

(57) **ABSTRACT**

The present disclosure provides a sintering assembly and a polycrystalline diamond compact (PDC) including a acid-labile leach-enhancing material, a PDC including cavities formed by removal of an acid-labile leach-enhancing material, and a method of forming a leached PDC using an acid-labile leach-enhancing material. The present disclosure further includes drill bits using PDCs formed suing an acid-labile leach-enhancing material.

**19 Claims, 11 Drawing Sheets**



|      |                         |                                                                                                                                                                                       |              |     |         |                  |              |
|------|-------------------------|---------------------------------------------------------------------------------------------------------------------------------------------------------------------------------------|--------------|-----|---------|------------------|--------------|
| (51) | <b>Int. Cl.</b>         |                                                                                                                                                                                       |              |     |         |                  |              |
|      | <i>E21B 10/55</i>       | (2006.01)                                                                                                                                                                             | 2007/0169419 | A1  | 7/2007  | Davis et al.     |              |
|      | <i>E21B 10/46</i>       | (2006.01)                                                                                                                                                                             | 2009/0313908 | A1  | 12/2009 | Zhang et al.     |              |
|      | <i>B22F 3/24</i>        | (2006.01)                                                                                                                                                                             | 2011/0024201 | A1* | 2/2011  | Scott .....      | E21B 10/573  |
|      | <i>B22F 7/06</i>        | (2006.01)                                                                                                                                                                             |              |     |         |                  | 175/428      |
|      | <i>C22C 26/00</i>       | (2006.01)                                                                                                                                                                             | 2012/0018223 | A1  | 1/2012  | Setlur et al.    |              |
| (52) | <b>U.S. Cl.</b>         |                                                                                                                                                                                       | 2012/0048626 | A1* | 3/2012  | Bellin .....     | E21B 10/5735 |
|      | CPC ....                | <i>E21B 10/5735</i> (2013.01); <i>B22F 2003/244</i> (2013.01); <i>B22F 2998/10</i> (2013.01); <i>B22F 2999/00</i> (2013.01); <i>E21B 10/46</i> (2013.01); <i>E21B 10/55</i> (2013.01) | 2013/0068540 | A1* | 3/2013  | DiGiovanni ..... | E21B 10/567  |
|      |                         |                                                                                                                                                                                       | 2013/0340352 | A1  | 12/2013 | Eve              | 175/430      |
|      |                         |                                                                                                                                                                                       | 2014/0013671 | A1  | 1/2014  | Belnap et al.    | 51/306       |
|      |                         |                                                                                                                                                                                       | 2014/0123565 | A1  | 5/2014  | Zhan et al.      |              |
|      |                         |                                                                                                                                                                                       | 2014/0165475 | A1  | 6/2014  | Lund             |              |
|      |                         |                                                                                                                                                                                       | 2015/0027787 | A1  | 1/2015  | Scott et al.     |              |
| (56) | <b>References Cited</b> |                                                                                                                                                                                       | 2016/0016291 | A1* | 1/2016  | Westraadt .....  | C04B 35/52   |
|      |                         |                                                                                                                                                                                       |              |     |         |                  | 51/297       |

## U.S. PATENT DOCUMENTS

8,328,891 B2 12/2012 Zhang et al.  
 8,435,317 B2 5/2013 Burgess et al.  
 8,470,060 B2 6/2013 Griffio et al.  
 8,535,400 B2 9/2013 Belnap et al.  
 8,679,206 B2 3/2014 Wan

## OTHER PUBLICATIONS

International Search Report received for PCT Patent Application No. PCT/US2016/060063, dated Jul. 13, 2017; 16 pages.

\* cited by examiner



FIG. 1A



FIG. 1B



FIG. 1C



FIG. 1D



FIG. 1E



FIG. 2A



FIG. 2B



FIG. 3A



FIG. 3B



FIG. 4A



FIG. 4B



FIG. 5



FIG. 6A



FIG. 6B



FIG. 7A



FIG. 7B



FIG. 9





FIG. 10

## 1

**POLYCRYSTALLINE DIAMOND COMPACT  
WITH INCREASED LEACHING SURFACE  
AREA AND METHOD OF LEACHING A  
POLYCRYSTALLINE DIAMOND COMPACT**

RELATED APPLICATIONS

This application is a U.S. National Stage Application of International Application No. PCT/US2016/060063 filed Nov. 2, 2016, which designates the United States, and is incorporated herein by reference in its entirety.

TECHNICAL FIELD

The current disclosure relates to a polycrystalline diamond compact (PDC), such as a cutter in an earth-boring drill bit.

BACKGROUND

Components of various industrial devices are often subjected to extreme conditions, such as high temperatures and high impact contact with hard and/or abrasive surfaces. For example, extreme temperatures and pressures are commonly encountered during drilling for oil extraction or mining purposes. Diamond, with its unsurpassed mechanical properties, can be the most effective material when properly used in a cutting element or abrasion-resistant contact element for use in drilling. Diamond is exceptionally hard, conducts heat away from the point of contact with the abrasive surface, and may provide other benefits in such conditions.

Diamond in a polycrystalline form has added toughness as compared to single-crystal diamond due to the random distribution of the diamond crystals, which avoids particular planes of cleavage from traversing the whole diamond thickness, such as, can be found in single-crystal diamond. Therefore, polycrystalline diamond is frequently the preferred form of diamond in many drilling applications. A drill bit cutting element that utilizes polycrystalline diamond is commonly referred to as a polycrystalline diamond compact (PDC) cutter. Accordingly, a drill bit incorporating PDC cutters may be referred to as a PDC bit.

PDCs can be manufactured in a cubic, belt, or other press by subjecting small grains of diamond and other starting materials to ultrahigh pressure and temperature conditions. One PDC manufacturing process involves forming a polycrystalline diamond table directly onto a substrate, such as a tungsten carbide substrate. The process involves placing a substrate containing a sintering aid, such as cobalt (Co), along with loose diamond grains mixed into a container of a press, and subjecting the contents of the press to a high-temperature high-pressure (HTHP) press cycle. The high temperature and pressure cause the small diamond grains to form into an integral polycrystalline diamond table intimately bonded to the substrate, with Co acting as sintering aid to promote the formation of new diamond-diamond bonds.

Although useful in creating the polycrystalline diamond table, sintering aids, such as Co, typically have a coefficient of thermal expansion (CTE), both linear and volumetric, significantly higher than that of diamond, such that, when the PDC heats up during use, remaining sintering aid material within polycrystalline diamond (PCD) expands more rapidly or to a greater degree than the diamond, sometimes causing cracks/micro cracks or otherwise modifying residual stresses within the diamond grains. A polycrystalline diamond table may be leached to remove at least a

## 2

portion of the sintering aid. The resulting leached PDC is more thermally stable than a similar, non-leached PDC. The resulting leached PDC is more thermally stable than a similar, non-leached PDC. Leached PDCs typically have at least 85% of the sintering aid removed. Leached PDCs may be leached to a given depth from the polycrystalline diamond outer surface, which is generally referred to as the leaching depth. The PDC may contain non-leached polycrystalline diamond, typically at a greater depth, for example, closer to the interface between the diamond table and the substrate.

Leaching large portions, or substantially all, of the sintering aid results in a thermally stable polycrystalline (TSP) diamond table. At a certain temperature, typically at least 750° C. at normal atmospheric pressure, the TSP cutters will not crack or graphitize, but non-leached PDCs will crack or graphitize under similar conditions. TSP diamond may be formed to a given leaching depth, or an entire diamond table may be TSP.

BRIEF DESCRIPTION OF THE DRAWINGS

A more complete understanding of the present embodiments and advantages thereof may be acquired by referring to the following description taken in conjunction with the accompanying drawings, which show particular embodiments of the current disclosure, in which like numbers refer to similar components, and in which:

FIG. 1A is a not-to-scale, cross-sectional schematic diagram of a sintering assembly for a PDC cutter with an acid-labile leach-enhancing material;

FIG. 1B is a not-to-scale, cross-sectional schematic diagram of a sintered PDC cutter with an acid-labile leach-enhancing material formed using the assembly of FIG. 1A;

FIG. 1C is a not-to-scale, cross-sectional schematic diagram of a sintered PDC cutter with increased leaching surface area formed by removal of acid-labile leach-enhancing material from the PDC cutter of FIG. 1B;

FIG. 1D is a not-to-scale, cross-sectional schematic diagram of a leached PDC cutter formed by leaching the sintered PDC cutter with increased leaching surface area of FIG. 1C;

FIG. 1E is a not-to-scale, cross-sectional schematic diagram of a backfilled PDC cutter formed by adding a backfill material to the leached PDC cutter of FIG. 1D;

FIG. 2A is a not-to-scale, cross-sectional schematic diagram of a sintering assembly for a PDC cutter with nanostructures of an acid-labile leach-enhancing material;

FIG. 2B is a not-to-scale, cross-sectional schematic diagram of a sintered PDC cutter with increased leaching surface area formed by removal of acid-labile leach-enhancing material from the nanostructures shown in FIG. 2A;

FIG. 3A is a not-to-scale, cross-sectional schematic diagram of a sintering assembly for a PDC cutter with both microstructures and nanostructures of an acid-labile leach-enhancing material;

FIG. 3B is a not-to-scale, cross-sectional schematic diagram of a sintered PDC cutter with increased leaching surface area formed by removal of acid-labile leach-enhancing material from the microstructures and nanostructures shown in FIG. 3A;

FIG. 4A is a not-to-scale, cross-sectional diagram of a sintering assembly for a PDC cutter with localized acid-labile leach-enhancing material;

FIG. 4B is a not-to-scale, cross-sectional diagram of a leached PDC cutter formed by removal of acid-labile leach-enhancing material shown in FIG. 4A to increase the leach-

ing surface area of the sintered PDC cutter, followed by leaching of the sintered PDC cutter;

FIG. 5 is a not-to-scale, cross-sectional diagram of a sintering assembly for a PDC cutter with a surface template of acid-labile leach-enhancing material;

FIG. 6A is a not-to-scale, cross-sectional diagram of a sintering assembly for a PDC cutter with a mesh template of acid-labile leach-enhancing material;

FIG. 6B is a not-to-scale, cross-sectional diagram of a sintered PDC cutter with increased leaching surface area formed by removal of the acid-labile leach-enhancing material shown in FIG. 6A;

FIG. 7A is a not-to-scale, cross-sectional diagram of a sintering assembly for a PDC cutter with two different acid-labile leach-enhancing materials;

FIG. 7B is a not-to-scale, cross-sectional diagram of a sintered PDC cutter with increase leaching surface area formed by removal of one, but not the other of the two different acid-labile leach-enhancing materials of FIG. 7A;

FIG. 8 is a series of not-to-scale, cross-sectional diagrams of various shapes of acid-labile leach-enhancing material in which:

FIG. 8A is an elongated microstructure or nanostructure;

FIG. 8B is a magnetic material-coated, elongated microstructure or nanostructure;

FIG. 8C is a template with an elongated microstructure or nanostructure having a terminal polarizable moiety;

FIG. 8D is a template material with dog-bone microstructures or nanosstructures;

FIG. 9 is a conceptual graph of leaching depth of a sintered PDC cutter versus days of leaching using conventional leaching in which the PDC cutter lacks increased leaching surface area formed by removal of an acid-labile leaching boost-material and for leaching using an acid-labile leach-enhancing material in a PDC cutter, as disclosed in the present disclosure, for forming increased leaching surface area formed by removal of an acid-labile leach-enhancing material; and

FIG. 10 is an earth-boring drill bit including at least one PDC in the form of a PDC cutter.

## DETAILED DESCRIPTION

The present disclosure relates to unleached PDCs with an acid-labile leach-enhancing material included in the polycrystalline diamond table. This acid-labile leach-enhancing material may be removed prior to or during leaching to increase the surface area of the polycrystalline diamond table available for further leaching. The present disclosure also includes leached PDCs containing cavities where acid-labile leach-enhancing material was located, or backfill material in such cavities. The present disclosure further provides methods of leaching the polycrystalline diamond table of a PDC using increased leaching surface area made available by removing acid-labile leach-enhancing material to leave cavities in the polycrystalline diamond table.

FIG. 1 is a series of cross-sectional schematic views of a sintering assembly used to form a PDC cutter with acid-labile leach-enhancing material through sintering, the PDC cutter with acid-labile leach-enhancing material, and the PDC cutter after removal of the acid-labile leach-enhancing material and after leaching and backfilling.

Referring to FIG. 1A, sintering assembly 10 includes can 20 containing substrate 30, diamond grains 40, and acid-labile leach-enhancing material 50. Sintering in a HTHP process results in sintered PDC cutter 70, as shown in FIG. 1B, that contains acid-labile leach-enhancing material 50 in

unleached polycrystalline diamond table 60a. Unleached polycrystalline diamond table 60a is bound to substrate 30.

In FIG. 1C, the acid-labile leach-enhancing material 50 has been removed, resulting in cavities 90 in unleached polycrystalline diamond table 60a. This produces sintered PDC cutter 80 with increased leaching surface area formed by the walls of cavities 90. Leaching then results in leached PDC cutter 100 as shown in FIG. 1D. Leached polycrystalline diamond table 60b in leached PDC cutter 100 may have both an unleached region 110, typically adjacent substrate 30, and leached region 120 surrounding cavities 90 and typically on the opposite side of the polycrystalline diamond table from substrate 30. As compared to a PDC with no acid-labile leach-enhancing material, the volume of the unleached region 110 will be smaller in the PDC shown in FIG. 1 and which utilizes acid-labile leach-enhancing material.

Leached PDC cutter 100 may be used without further treatment. However, cavities 90 may also be wholly or partially filled with a backfill material 140 to result in backfilled PDC cutter 130, as shown in FIG. 1E. Backfill material may include silicon (Si) or a carbide-forming element, such as tungsten (W). Backfilling may increase the impact toughness or other mechanical properties of back-filled PDC cutter 130 as compared to leached PDC cutter 100.

Substrate 30 may be any substrate suitable for use in a PDC cutter. In particular, it may be a conventional substrate, such as a tungsten carbide substrate. Substrate 30 may include a sintering aid that catalyzes the formation of diamond-diamond bonds, allowing diamond grains 40 to form polycrystalline diamond table 60 in the HTHP process. The sintering aid may also be located with diamond grains 40, both in substrate 30 and diamond grains 40, or in any other location that allows it to catalyze the formation of diamond-diamond bonds during the HTHP process. The sintering aid may also assist in bonding diamond table 60 to substrate 30 and in forming substrate 30 if it is not in final form before the HTHP process. Any one or combination of sintering aids may be used. Suitable sintering aids include Group VIII metals, such as Co, nickel (Ni), iron (Fe), or copper (Cu), and their alloys.

Diamond grains 40 may be any suitable diamond grains, including diamond grains of substantially uniform grain sizes, diamond grains of mixed grain sizes, or mixtures thereof located in different areas of what will become polycrystalline diamond table 60 after it is formed.

Acid-labile leach-enhancing material 50 may be any material that is able to remain at least partially intact during the HTHP process and then be dissolved by acid more readily than at least one sintering aid because it is more acid-labile in the acid than the sintering aid. The purpose of acid-labile leach-enhancing material 50 is to be removed by acid prior to or during leaching, thereby forming cavities 90, which provide greater surface area of polycrystalline diamond table 60 in contact with a leaching fluid. Accordingly, acid-labile leach-enhancing material 50 may be dissolved by acid more readily than all sintering aids, when more than one sintering aid is present, because it is more acid-labile in the acid than any of the sintering aids.

Suitable acid-labile leach-enhancing materials 50 include W, hafnium (Hf), and vanadium (V), metal-coated W, Hf, or V, such as Ni or Co-coated W, Hf, or V, and other metals or alloys, ceramics, and glasses.

In order to remain at least partially intact during the HTHP process, suitable acid-labile leach-enhancing materials 50 may have limited ability to dissolve into or otherwise

enter diamond grains **40** during an HTHP process. They may also be able to retain their general shape during such a process. Thus, at least a portion of the acid-labile leach-enhancing material **50** will typically have a melting point above the temperature of the HTHP process. Acid-labile leach-enhancing materials **50** may have sufficient ductility to cause them to elongate during an HTHP process, thereby further increasing leaching surface area provided by cavities **90**.

Acid-labile leach-enhancing materials **50** may be removed by a pre-leaching acid prior to leaching polycrystalline diamond table **60**. A pre-leaching acid may be able to remove at least 80 wt %, at least 90 wt %, at least 95 wt %, or at least 99 wt % of acid-labile leach-enhancing materials **50** when incubated at 20° C. for 1 day. The pre-leaching acid may also remove no more than 10 wt % of the sintering aid from polycrystalline diamond table **60a** when incubated at 20° C. for 1 day, although in most instances, removal of sintering aid during pre-leaching is not a problem and may actually be a benefit, such that it is not a concern of more than 10 wt % sintering aid is removed by the pre-leaching acid.

Hydrofluoric acid (HF) is an example of one suitable pre-leaching acid for use with a W-containing acid-labile leach-enhancing material **50**.

Leaching may then be conducted with any suitable leaching agent able to dissolve at least one sintering aid and remove it from polycrystalline diamond table **60**. For instance, nitric and sulfuric acids and mixtures thereof are often used as the leaching agent for Co and Co-based sintering aids. Leached agents enter polycrystalline diamond via a surface in contact with the leaching agent and leached sintering aid exits with such a surface. The surface area of a polycrystalline diamond table available to contact the leaching agent may be referred to as the leaching surface area. Cavities **90** increase the leaching surface area of polycrystalline diamond table **60**. In particular, cavities **90** increase the leaching surface area inside polycrystalline diamond table **60**.

In FIG. 1D and FIG. 1E, leached polycrystalline diamond table **60b** refers to any polycrystalline diamond table that has had sintering agent removed by a leaching agent. Although FIG. 1D and FIG. 1E depict a distinct leached portion **120** and unleached portion **110** of leached polycrystalline diamond table **60b** with a sharp boundary between the portions, this depiction is for ease of understanding the basic concept only. Actual leached PDC cutters typically have a gradual transition from a portion where substantial amounts of sintering aid have been removed to a portion where most or all sintering aid remains.

Although FIG. 1 depicts the progression of a PDC cutter through a pre-leaching step and a separate leaching step, the leaching agent typically can also dissolve acid-labile leach-enhancing material **50**, such that the pre-leaching step may be omitted. In such instances, removal of acid-labile leach-enhancing material **50** and leaching may occur concurrently, such that cavities **90** increase in size while leaching occurs.

In addition, although FIG. 1 and other figures herein depict acid-labile leach-enhancing material **50** as either wholly present or entirely absent, often some acid-labile leach-enhancing material **50** may remain in polycrystalline diamond table **60**, even after leaching because it is difficult to remove all of any type of material from polycrystalline diamond table **60**. In some instances, acid-labile leach-enhancing material **50** may intentionally be left in polycrystalline diamond table **60**. For example, a process may be used in which some acid-labile leach-enhancing material **50**

is removed and polycrystalline diamond table **60** is leached, then the leaching profile may be evaluated to determine if more acid-labile leach-enhancing material removal and leaching is needed to obtain a PDC cutter with a particular leaching profile. If further leaching is not needed, then some acid-labile leach-enhancing material **50** may be left in the PDC cutter. Such remaining material may provide mechanical strength as well as impact toughness to the PDC cutter.

Acid-labile leach-enhancing material **50** may be in the form of microstructures or nanostructures, or a mixture thereof. Microstructures generally have an average largest linear dimension of at least 1 μm and less than 1000 μm, less than 500 μm, or less than 100 μm. Nanostructures generally have an average largest linear dimension of at least 1 nm and less than 1000 nm, less than 500 nm, or less than 100 nm. Microstructures may be better able to increase leaching surface area than nanostructures, but microstructures may cause greater decreases in mechanical strength of polycrystalline diamond table **60** than do nanostructures. Due to the tendency of microstructures to decrease mechanical strength of polycrystalline diamond table **60** more than nanostructures, it may be possible to include more acid-labile leach-enhancing material **50** by overall volume when it is in the form of nanostructures. Thus, the total available leaching surface area may still be similar to that obtained using microstructures.

FIG. 1 depicts acid-labile leach-enhancing material **50** in the form of microstructures. These microstructures are oriented in a pattern among diamond grains **40** in FIG. 1A. After the HTHP process and removal of acid-labile leach-enhancing material **50**, resulting cavities **90** are in a similar pattern in polycrystalline diamond table **90**, as shown in FIGS. 1B-1D. In the pattern shown, each element **50** may extend into polycrystalline diamond table **60** from the adjacent surface at least 1 μm, at least 10 μm, at least 50 μm, at least 100 μm, or at least 200 μm, or another distance within 1 μm or 5 μm of the leaching depth. The leaching surface area of unleached polycrystalline diamond table **60a** in FIG. 1C or other polycrystalline diamond tables formed using microstructures of acid-labile leach-enhancing material **50** may be at least 10% greater, at least 30% greater, or at least 50% greater than in an otherwise identical polycrystalline diamond table lacking cavities **90**.

FIG. 2A depicts acid-labile leach-enhancing material **50** in the form of nanostructures. These nanostructures are dispersed in a portion of diamond grains **40**. After the HTHP process and removal of acid-labile leach-enhancing material **50**, resulting cavities **90** are in a similar portion of polycrystalline diamond table **60**, as shown in FIG. 2B. That portion of polycrystalline diamond table **60** may extend from the adjacent surface at least 1 μm, at least 10 μm, at least 50 μm, at least 100 μm, or at least 200 μm, or another distance within 1 μm or 5 μm of the leaching depth. The leaching surface area of the unleached polycrystalline diamond table formed using nanostructures of acid-labile leach-enhancing material may be at least 5% greater, at least 10% greater, or at least 20% greater than in an otherwise identical polycrystalline diamond table lacking cavities.

The benefits of both microstructures and nanostructures of acid-labile leach-enhancing material **50** may be achieved by using a mixture of both. The proportions of microstructures to nanostructures by number in the mixture may be between 5:1 and 1:5, in particular between 2:1 and 1:2. FIG. 3A depicts sintering assembly **10** containing both acid-labile leach-enhancing material **50a** in the form of microstructures and acid-labile leach-enhancing material **50b** in the form of nanostructures. After sintering, in the PDC cutter of FIG.

3B, microstructure cavities **90a** may allow the leaching agent to readily penetrate to a given depth from the surface of polycrystalline diamond table **60**, while the nanostructure cavities **90b** may facilitate movement of the leaching agent out from microstructure cavities **90a**. The portion of polycrystalline diamond table **60** in which acid-labile leach-enhancing material **50** is found may extend from the adjacent surface at least 1  $\mu\text{m}$ , at least 10  $\mu\text{m}$ , at least 50  $\mu\text{m}$ , at least 100  $\mu\text{m}$ , or at least 200  $\mu\text{m}$ , or another distance within 1  $\mu\text{m}$  or 5  $\mu\text{m}$  of the leaching depth. The leaching surface area of the unleached polycrystalline diamond table formed using a combination of microstructures and nanostructures of acid-labile leach-enhancing material may be at least 10% greater, at least 30% greater, at least 50% greater, or at least 60% greater than in an otherwise identical polycrystalline diamond table lacking cavities.

Acid-labile leach-enhancing material **50**, whether in the form of microstructures, nanostructures, or a mixture, may be evenly distributed within diamond grains **40** so that cavities **90** are evenly distributed within polycrystalline diamond table **60** or a portion thereof. This even distribution may increase the mechanical stability of polycrystalline diamond table **60**, particularly if cavities **90** are not back-filled.

Although FIGS. 1-3 depict acid-labile leach-enhancing material that reaches to a leaching depth from a top surface of the PDC cutter, the leaching depth may also extend from a side surface if, as depicted in FIG. 4A, acid-labile leach-enhancing material **50** is placed along the upper and side portions of diamond grains **40** in sintering assembly **10**. After the HTHP process and leaching, leached polycrystalline diamond table **60b** of FIG. 4B contains a leached portion **120** on the top and sides, and a central unleached portion **110**.

Acid-labile leach-enhancing material **50** may be oriented in diamond grains **40** and subsequently in polycrystalline diamond table **60** in a particular pattern or manner. For instance, elongated microstructures of acid-labile leach-enhancing material **50**, such as those of FIG. 1 may be oriented so that they extend lengthwise into polycrystalline diamond table **60** from, at, or near its surface, particularly its top surface. This allows the leaching agent to readily penetrate to a depth within polycrystalline diamond table **60** and thus readily leach to at least that depth.

In addition because fractures in the polycrystalline diamond table during PDC use tend to run along boundaries between leached and unleached regions, acid-labile leach-enhancing material **50** may be oriented in a particular pattern or manner to direct the location of such boundaries and thus the likely location of fractures, which may lead to improved PDC life.

Acid-labile leach-enhancing material **50** may be oriented using any of a variety of methods. For instance, if acid-labile leach-enhancing material **50** contains a magnetic component, such as a Co, Ni, or Fe coating on W as shown in FIG. 8B or an internal magnetic component, then a magnetic field may be used to orient the material. Acid-labile leach-enhancing material **50** may also contain a polarizable moiety, such as that shown in FIG. 8C, which allows an electric field to be used to orient it.

Acid-labile leach-enhancing material **50** may also be directed to particular regions of diamond grains **40** and ultimately polycrystalline diamond table **60** using a magnetic or electric field, or by vibrating sintering assembly **10**.

As shown in FIG. 5, acid-labile leach-enhancing material **50** may also be formed on a template, such as template **150**. This template may be made from the acid-labile leach-

enhancing material, which may facilitate its removal from unleached polycrystalline diamond table **60a**. It may also include any material that does not interfere with the HTHP process. For instance template **150** may include a polymer binder that largely decomposes to carbon (C) during the HTHP process. If template **150** includes a material that does interfere with the HTHP process, then it may further include a sink material that absorbs the interfering material.

Acid-labile leach-enhancing material **50** may be grown on or with template **150**. It may also be 3-D printed using additive manufacturing on or with template **150**.

Rather than using a separate template **150**, acid-labile leach-enhancing material **50** may also simply be adhered to or grown on can **20**.

Regardless of the template **150** used or whether the acid-labile leach-enhancing material **50** is grown on can **20**, after removal and leaching, a leached polycrystalline diamond table **60b** similar to that of FIG. 1D may be obtained.

Pre-formed structures of acid-labile leach-enhancing material **50** may also be used within diamond grains **40** prior to sintering, resulting in cavities **90** with a particular orientation in polycrystalline diamond table **60**. For instance, as shown in FIG. 6A, acid-labile leach-enhancing material **50** may be in the form of a mesh placed in diamond grains **40**. This results in a mesh-pattern of cavities in polycrystalline diamond table **90**, as shown in FIG. 6B. Although the mesh of FIG. 6 is shown encompassing a large contiguous area and in an orientation perpendicular to the top surface of the polycrystalline diamond table **60**, the mesh may be located in smaller contiguous area, or a plurality of meshes may be in a plurality of non-contiguous areas to enhance mechanical stability of the polycrystalline diamond table. In addition, the mesh may be in any orientation with respect to any part of the PDC cutter. For instance, it may be parallel to the top surface of the polycrystalline diamond table **60**, or there may be a plurality of meshes in a plurality of orientations.

Although a mesh may be formed having either a micro- or nano-sized diameter of its component strands, nano-sized strands may be more effective.

A mesh of acid-labile leach-enhancing material **50** results in an interconnected grid or a plurality of interconnected grids of cavities **90**. However, acid-labile leach-enhancing material **50** may also form an interconnected grid or plurality of interconnected grids of cavities **90** in other manners.

For instance, microstructures and nanostructures may be arranged such that they occasionally touch one another, which produces connected cavities **90**. This may be particularly effective when a combination of both microstructures **50a** and nanostructures **50b** of acid-labile leach-enhancing material are used, as shown in FIG. 3A. This results in an interconnected grid or plurality of interconnected grids of cavities **90**, as shown in FIG. 3B, with the microstructure cavities **90a** oriented with respect to the surface to allow penetration of the leaching agent to a depth within polycrystalline diamond table **60**, and at least some nanostructure cavities **90b** interconnecting at least some microstructure cavities **90a**.

Multiple ways of orienting or directing acid-labile leach-enhancing material **50** may be employed to produce the same PDC cutter. For instance, elongated nanostructures of acid-labile leach-enhancing material **50** having polarizable terminal moieties, such as those shown in FIG. 8C, may be grown on can **20**, then subjected to an electric field to further orient them into diamond grains **40**. In another example, microstructures of acid-labile leach-enhancing material **50** may be formed on a template **150** as shown in FIG. 5, and nanostructures of acid-labile leach-enhancing material **50**

may be mixed into all or a region of diamond grains **40** so that, as a whole, acid-labile leach-enhancing material **50** contains both microstructures and nanostructures. In still another example, microstructures of acid-labile leach-enhancing material **50a** may be oriented as shown in FIG. 3A using a magnetic or electric field, but nanostructures of acid-labile leach-enhancing material **50b** may be mixed into all or a region of diamond grains **40** and may remain that way even when microstructures **50a** are oriented because nanostructures **50b** are not responsive to the magnetic or electric field.

More than one type of acid-labile leach-enhancing material **50** may be used to form a single PDC cutter. These multiples types of material may be mixed together uniformly or in different proportions, then placed in diamond grains **40**. Alternatively, the different types of materials may be localized to different regions of diamond grains **40**. For instance, a first, more acid-labile leach-enhancing material **50c** may be placed around the circumference of the chamber containing diamond grains **40**, while a second less acid-labile leach-enhancing material **50d** may be placed in a central portion of the chamber, as shown in FIG. 7A. A first pre-leaching agent may be used to remove the first acid-labile leach-enhancing material **50c**, followed by leaching. This results in a PDC cutter **160** as shown in FIG. 7B, with cavities **90** and a leached portion **120** of polycrystalline diamond table **60b** around the circumference of polycrystalline diamond table and second acid-labile leach-enhancing material **50d** in a central unleached portion **110** of polycrystalline diamond table **60b**. PDC cutter may be used in this configuration. However, a different PDC cutter may be readily produced from the same unleached polycrystalline diamond table by simply using a second pre-leaching agent that removes both acid-labile leach-enhancing materials **50c** and **50d**, resulting in a PDC cutter **100** as shown in FIG. 1D.

Although the acid-labile leach-enhancing material **50** of FIGS. 1-7 is shown in an elongated shape, it may have any shape. A free-standing elongated microstructure or nanostructure of acid-labile leach-enhancing material is shown in FIG. 8A. Such as structure may also be incorporated into a template, attached to the can, or formed into a mesh or otherwise incorporated into a larger structure.

FIG. 8B is a magnetic material-coated, elongated microstructure or nanostructure of acid-labile leach-enhancing material **50**. The structure contains magnetic material coating **170**. Although any magnetic material may be used, if it is also a sintering aid, such as Co, Fe, or Ni, then it may be used to orient the acid-labile leach-enhancing material **50** prior to sintering, then at least partially disperse from the acid-labile leach-enhancing material **50** during the HTHP process and act as a sintering aid. Alternatively if the magnetic material is located internally within acid-labile leach-enhancing material **50**, then it may be largely sequestered until the pre-leaching agent is applied, such that it does not participate in or interfere with diamond table formation during the HTHP process. A free-standing elongated microstructure or nanostructure of acid-labile leach-enhancing material is shown in FIG. 8B. Such as structure may also be incorporated into a template, attached to the can, or formed into a mesh or otherwise incorporated into a larger structure.

FIG. 8C is a template **150** with an elongated microstructure or nanostructure of acid-labile leach-enhancing material **50** having a terminal polarizable moiety **180**. Such an elongated microstructure or nanostructure of acid-labile

leach-enhancing material **50** may also be free-standing, formed on or adhered to the can, or otherwise incorporated into a larger structure.

FIG. 8D is a template material **150** with dog-bone microstructures or nanostructures of acid-labile leach-enhancing material **190**. These structures have enlarged edges that increase the overall surface area of cavities **90** as compared to cavities formed from more cylindrical structures. Microstructures or nanostructures **190** may be formed by plating the acid-labile leach-enhancing material on template material **150**. They may also be formed by plating acid-labile leach-enhancing material on the interior of a can. Pronounced edges and corners result from the higher current density in those locations during a plating process. Although FIG. 8D illustrates a template in which a coating is plated, other variations are possible.

In addition to the sintering assemblies and PDC cutters described in FIGS. 1-7, the present disclosure further provides a method of forming a leached PDC cutter. The method generally uses and results in the structures shown in FIGS. 1A-E.

A substrate and polycrystalline diamond power with acid-labile leach-enhancing material are combined in a can to form a sintering assembly that is subjected to an HTHP process that forms a sintered PDC cutter with an unleached polycrystalline diamond table in which the acid-labile leach-enhancing material remains at least partially intact. The unleached polycrystalline diamond is then placed in a pre-leaching agent that removes at least a portion of the acid-labile leach-enhancing material to form cavities in the polycrystalline diamond table of the sintered PDC cutter. The PDC cutter is then placed in a leaching agent that removes a sintering aid from the polycrystalline diamond table to form a leached polycrystalline diamond table in a leached PDC cutter. The leached polycrystalline diamond table may still have leached and unleached portions. In particular, it may have a leached portion extending to a leaching depth from a surface, and an unleached portion adjacent the substrate. The cavities remain in the leached polycrystalline diamond table after leaching, but they may be backfilled with a backfill material to produce a backfilled PDC cutter.

When conventional leaching methods are used, the rate of leaching slows down as leaching progresses to greater depths within the PDC cutter. Thus, the rate of leaching also slows down as total leaching time increases. This effect is illustrated conceptually by the "Conventional Leaching" line in the graph of FIG. 9. Using the structures and methods described herein, the leaching rate may be slowed to a lesser extent as leaching progresses to greater depths and as total time increases. This effect is illustrated conceptually by the "Leach-enhancing Material" line in the graph of FIG. 9. As the graph of FIG. 9 also illustrates, when the structures and methods described herein are used, a given leaching depth may be achieved in less time than with conventional methods. Alternatively, when the structures and methods described herein are used, a greater leaching depth may be achieved in the same time as with conventional methods.

A PDC cutter as described herein or formed using the methods described herein may be incorporated into an industrial device, such as an earth-boring drill bit, as illustrated in FIG. 10. FIG. 10 illustrates a fixed cutter drill bit **200** containing a plurality of cutters **210** coupled to drill bit body **220**. At least one of cutters **210** may be a leached PDC cutter or a backfilled PDC cutter as described herein.

Bit body **220** may include a plurality of blades **230** extending therefrom. Bit body **220** may be formed from

## 11

steel, a steel alloy, a matrix material, a metal-matrix composite, or other suitable bit body material desired strength, toughness and machinability. Bit body 220 may be formed to have desired wear and erosion properties. PDC cutters 210 may be located in gage region 240, or in a non-gage region, or both.

Drilling action associated with drill bit 200 may occur as bit body 220 is rotated relative to the bottom of a wellbore in response to rotation of an associated drill string. At least some PDC cutters 210 disposed on associated blades 230 may contact adjacent portions of a downhole formation during drilling. These PDC cutters 210 may be oriented such that their polycrystalline diamond tables contact the formation.

The present disclosure provides an embodiment A relating to an unleached PDC including a substrate and an unleached polycrystalline diamond table including an acid-labile leach-enhancing material and a sintering aid.

The present disclosure provides an embodiment B relating to a leached PDC including a substrate and a leached polycrystalline diamond table including a plurality of microstructure or nanostructure cavities, or a mixture thereof.

The present disclosure provides an embodiment C relating to a drill bit including a bit body and the PDC of embodiment B.

The present disclosure provides an embodiment D relating to a PDC sintering assembly including a substrate, polycrystalline diamond grains, a sintering aid, microstructures or nanostructures or a mixture thereof of acid-labile leach-enhancing material disposed in the polycrystalline diamond grains, and a can in which the substrate, polycrystalline diamond grains, sintering aid and acid-labile leach-enhancing material are disposed.

The present disclosure further provides an embodiment E relating to a method of forming a leached PDC by placing a substrate, polycrystalline diamond grains containing microstructures, nanostructures, or a mixture of both of an acid-labile leach-enhancing material, and a sintering aid in a can to form a sintering assembly, performing an HTHP process on the sintering assembly to produce a sintered PDC with a polycrystalline diamond table containing the acid-labile leaching boost material, removing at least a part of the acid-labile leach-enhancing material from the polycrystalline diamond table, and leaching the polycrystalline diamond table to remove at least a part of the sintering aid.

In addition, embodiments A, B, C, D and E may be used in conjunction with one another and the following additional elements, which may also be combined with one another unless clearly mutually exclusive, and which method elements may be used to obtain devices and which device elements may result from methods: i) the acid-labile leach-enhancing material may be more labile in an acid than the sintering aid; ii) the acid-labile leach-enhancing material may be in the form of a microstructure; iii) the acid-labile leach-enhancing material may be in the form of a nanostructure; iv) the acid-labile leach-enhancing material may be in a dog bone structure; v) the acid-labile leach-enhancing material may be coated with a magnetic material; vi) the acid-labile leach-enhancing material may have a polarizable moiety; vii) the acid-labile leach-enhancing material may be part of a template; viii) the acid-labile leach-enhancing material may be part of a mesh; ix) the acid-labile leach-enhancing material may be adhered to the can; the acid-labile leach-enhancing material may be oriented in a pattern in the polycrystalline diamond table; x) the acid-labile

## 12

leach-enhancing material may be may include W; x) the acid-labile leach-enhancing material may define a plurality of cavities within the polycrystalline diamond table that increase the leaching surface area of the polycrystalline diamond table after removal of the acid-labile leach-enhancing material; xi) the polycrystalline diamond table may include a plurality of both microstructure and nanostructure cavities; xii) the microstructure or nanostructure cavities, or both, form at least one interconnected grid of cavities; xiii) the microstructure or nanostructure cavities may increase the leaching surface area of the polycrystalline diamond table; ix) the cavities may include a backfill material; x) the leached polycrystalline diamond may include a leached region surrounding the plurality of cavities and an unleached region; xi) the substrate may include the sintering aid; xii)

Although only exemplary embodiments of the invention are specifically described above, it will be appreciated that modifications and variations of these examples are possible without departing from the spirit and intended scope of the invention. For instance, the use of PDCs on other industrial devices may be determined by reference to the drill bit example.

What is claimed is:

1. An unleached polycrystalline diamond compact (PDC) comprising:

a substrate; and

an unleached polycrystalline diamond table including an acid-labile leach-enhancing material and a sintering aid, wherein the acid-labile leach-enhancing material is more labile in an acid than the sintering aid and comprises a mixture of both of microstructures having an average largest linear dimension of less than 100  $\mu\text{m}$  and nanostructures having an average largest linear dimension of less than 1000 nm.

2. The PDC of claim 1, wherein the sintering aid comprises cobalt and the acid-labile leach-enhancing material comprises tungsten (W).

3. The PDC of claim 1, wherein the acid-labile leach-enhancing material is configured for removal in the acid to define a plurality of cavities of less than 100  $\mu\text{m}$  within the polycrystalline diamond table that increase the leaching surface area of the polycrystalline diamond table as a result of the removal of the acid-labile leach-enhancing material.

4. An unleached polycrystalline diamond compact (PDC) comprising:

a substrate; and

an unleached polycrystalline diamond table including an acid-labile leach-enhancing material and a sintering aid, wherein the acid-labile leach-enhancing material is more labile in an acid than the sintering aid and comprises one or both of microstructures having an average largest linear dimension of less than 100  $\mu\text{m}$  and nanostructures having an average largest linear dimension of less than 1000 nm, wherein one or both of the microstructures and the nanostructures of the acid-labile leach-enhancing material are oriented in a pattern in the polycrystalline diamond table.

5. The PDC of claim 4, wherein the sintering aid comprises cobalt and the acid-labile leach-enhancing material comprises tungsten (W).

6. The PDC of claim 4, wherein the acid-labile leach-enhancing material is in the form of a mixture of both the microstructures and the nanostructures.

7. The PDC of claim 4, wherein the acid-labile leach-enhancing material is configured for removal in the acid to define a plurality of cavities of less than 100  $\mu\text{m}$  within the polycrystalline diamond table that increase the leaching

**13**

surface area of the polycrystalline diamond table as a result of the removal of the acid-labile leach-enhancing material.

**8.** A polycrystalline diamond (PDC) sintering assembly comprising:

- a substrate;
- polycrystalline diamond grains;
- a sintering aid;
- one or both of microstructures having an average largest linear dimension of less than 100  $\mu\text{m}$  or nanostructures having an average largest linear dimension of less than 1000 nm of an acid-labile leach-enhancing material disposed in the polycrystalline diamond grains, wherein the acid-labile leach-enhancing material is oriented in a pattern in the polycrystalline diamond grains; and
- a can in which the substrate, polycrystalline diamond grains, sintering aid, and acid-labile leach-enhancing material are disposed.

**9.** The PDC sintering assembly of claim **8**, wherein the substrate comprises the sintering aid.

**10.** The PDC sintering assembly of claim **8**, wherein the acid-labile leach-enhancing material is more labile in an acid than the sintering aid.

**11.** The PDC sintering assembly of claim **8**, wherein the acid-labile leach-enhancing material comprises tungsten (W).

**12.** A polycrystalline diamond (PDC) sintering assembly comprising:

- a substrate;
- polycrystalline diamond grains;
- a sintering aid;
- one or both of microstructures having an average largest linear dimension of less than 100  $\mu\text{m}$  or nanostructures having an average largest linear dimension of less than 1000 nm of an acid-labile leach-enhancing material disposed in the polycrystalline diamond grains, wherein the acid-labile leach-enhancing material has a dog-bone structure; and

**14**

a can in which the substrate, polycrystalline diamond grains, sintering aid, and acid-labile leach-enhancing material are disposed.

**13.** The PDC sintering assembly of claim **12**, wherein the substrate comprises the sintering aid.

**14.** The PDC sintering assembly of claim **12**, wherein the acid-labile leach-enhancing material is more labile in an acid than the sintering aid.

**15.** The PDC sintering assembly of claim **12**, wherein the acid-labile leach-enhancing material comprises tungsten (W).

**16.** A polycrystalline diamond (PDC) sintering assembly comprising:

- a substrate;
- polycrystalline diamond grains;
- a sintering aid;
- one or both of microstructures having an average largest linear dimension of less than 100  $\mu\text{m}$  or nanostructures having an average largest linear dimension of less than 1000 nm of an acid-labile leach-enhancing material disposed in the polycrystalline diamond grains, wherein the acid-labile leach-enhancing material is in the form of a template or mesh or adhered to the can; and

a can in which the substrate, polycrystalline diamond grains, sintering aid, and acid-labile leach-enhancing material are disposed.

**17.** The PDC sintering assembly of claim **16**, wherein the substrate comprises the sintering aid.

**18.** The PDC sintering assembly of claim **16**, wherein the acid-labile leach-enhancing material is more labile in an acid than the sintering aid.

**19.** The PDC sintering assembly of claim **16**, wherein the acid-labile leach-enhancing material comprises tungsten (W).

\* \* \* \* \*